

# UNITED STATES PATENT OFFICE.

GRENVILLE MELLEN, OF MOUNT VERNON, NEW YORK.

## PROCESS OF MELTING ALUMINUM OR ALUMINUM ALLOYS

1,160,430.

Specification of Letters Patent. Patented Nov. 16, 1915.

No Drawing.

Application filed February 10, 1911. Serial No. 607,864.

To all whom it may concern:

Be it known that I, GRENVILLE MELLEN, citizen of the United States, and resident of Mount Vernon, in the county of Westchester and State of New York, have invented certain new and useful Improvements in Processes of Melting Aluminum or Aluminum Alloys, of which the following is a specification.

10 This invention relates to a new and useful process of melting aluminum and its alloys and has for its object to protect and preserve the metal from destruction by oxidation and to produce ingot and other forms 15 of casting which shall be of a sounder nature to a degree that has been heretofore practically impossible to effect.

It is of course well understood by those familiar with the practice of melting aluminum or its alloys that while it would be 20 extremely desirable to produce ingot or other forms of castings which shall be practically devoid of the tendency to "blow-holes" and other causes of imperfection 25 which are due to the presence of numerous bubbles of gas disbursed throughout the mass, it has been found practically impossible to produce metal which has undergone the present method of melting aluminum or 30 its alloys, and having these qualities to the desired extent. It is also extremely desirable to obtain a process or method of melting aluminum or its alloys which shall preserve the metal from the great loss suffered 35 by oxidation.

It is generally known that if molten aluminum or any of its alloys is allowed to remain within the furnace, and the temperature gradually raised, the deterioration of 40 the metal increases with the rise of the temperature. Numerous "blow-holes" occur when the metal is cast. If the metal is melted with care and skill, of course, many of these imperfections are avoided. But 45 with the present methods and processes of melting aluminum or its alloys, the results are far from being satisfactory even if the greatest care is taken by the most skilled hands. The imperfections are inevitable so 50 long as the cause remains; and the causes of these difficulties with the present methods of melting aluminum or its alloys are ever present.

In the melting of "scrap" aluminum 55 (this aluminum is in the majority of cases selāom even commercially pure, it being

generally an aluminum alloy with copper, sometimes zinc, either or both, and occasionally, though rarely containing other elements), which consist of "clippings" and "stampings" of the sheet metal (generally purer aluminum than that which composes the castings), and the "turnings", "grindings", and "filings" which are parts of the alloys which are adapted to the casting requirements, a great loss is suffered through oxidation. This loss, is generally less in the metals whose compositions more nearly approach pure aluminum. The percentage of loss suffered by these at present varies between ten and forty. It is in the case of the "turnings", "clippings", and "filings" that the greatest loss is suffered; the loss ranging between twenty-five and forty per cent. of the whole. In practice this great loss is seldom less than thirty per cent. This loss is practically a total destruction and an absolute waste of valuable metal.

In the instance of the imperfections arising from the "blow-holes" and the like, I have found that this is due to the presence of occluded gases, and to the partial dissolution of the oxids, and other foreign and injurious matter.

In the case of the great loss by oxidation, I have found that this is due to the presence of oxygen, which exists free as a constituent of the air, and in the water vapor which is present in the atmosphere. It is generally known that aluminum decomposes water vapor, forming the oxid of aluminum and liberating the two atoms of hydrogen.

My novel process overcomes these difficulties, and produces the metal with the tendency to "blow-holes" and gas bubbles practically obviated. It also preserves the metal to a minimum loss by oxidation; the percentage of loss being reduced to between one-half and five.

With these and other objects in view, I have made numerous experiments in the melting of aluminum and its alloys, and both of these are in the form of "scrap".

It is readily obvious that matter existing in the forms of "scrap-aluminum," and the "scrap" of aluminum alloys exposes a surface area which bears a great numerical proportion to the entire volume of the mass. Therefore a large portion of the metal exists in intimate contact with the oxygen present in the atmosphere. This same surface is exposed to the number of gases which con-

stitute the atmosphere within the furnace. This atmosphere generally contains carbon dioxid, sulfur-dioxid, water-vapor, free oxygen, free nitrogen, and some free hydro-  
gen. All metals will occlude gas under cer-  
tain conditions, though each may show some  
partiality as to the nature of the gas.

In carrying out my novel process I prefer  
to use either of the following methods: The  
10 aluminum or the aluminum alloy to be melt-  
ed is placed in a crucible or in any suitable  
melting chamber which is inclosed in an air  
tight chamber. The air is then removed  
from the said air tight chamber, thus creat-  
15 ing a partial vacuum therein. Any inert  
gas is now admitted into the said air-tight  
chamber. The metal is melted in this atmos-  
phere. The object of this inert gas is to pro-  
vide an atmosphere which shall serve as a  
20 means of conducting the heat to all parts of  
the metal not in direct contact with the heat-  
ed walls of the said crucible or melting  
chamber, and to provide an atmosphere  
which shall be free from active oxygen or  
25 other corrosive gases which act upon alum-  
num or aluminum alloys. After the metal is  
melted in this inert atmosphere and while  
the metal is yet molten, the inert gas is re-  
moved, thus again creating a partial vacuum  
30 within the said air-tight chamber.

The molten metal is allowed to remain  
therein until much of the occluded gas is ex-  
pelled from the pores of the aluminum or  
the aluminum alloy. The metal is then  
35 ready for pouring which should be done as  
quickly as possible to prevent the further  
occlusion of gas.

In the melting of aluminum or aluminum  
alloys to prevent the occlusion of gases by  
40 the metal and to prevent its great loss by  
oxidation, if preferred the metal may be  
placed in a crucible or other suitable melt-  
ing chamber, the whole inclosed within an  
airtight chamber and the air removed from  
45 within the said airtight chamber, thus cre-  
ating a partial vacuum therein, and the  
metal melted therein. The aluminum or the  
aluminum alloy is in this way melted in the  
atmosphere of a partial vacuum.

50 Having thus described my invention, I  
claim:

1. The process of melting aluminum or an

aluminum alloy which consists in melting  
the aluminum or the aluminum alloy in  
the atmosphere of a gas substantially chem-  
ically inert toward the aluminum or the  
55 aluminum alloy, then creating a partial  
vacuum within the melting chamber while  
the aluminum or the aluminum alloy is yet  
molten.

2. The process of melting aluminum or an  
aluminum alloy which consists in creating a  
partial vacuum within the melting chamber,  
then admitting a gas which is substantially  
chemically inert toward the aluminum or the  
65 aluminum alloy into the melting chamber,  
and then melting the aluminum or the alum-  
num alloy in this atmosphere which is sub-  
stantially chemically inert toward the  
aluminum or the aluminum alloy.

3. The process of melting aluminum or an  
aluminum alloy which consists in creating a  
partial vacuum within the melting cham-  
ber, then admitting a gas which is substan-  
tially chemically inert toward the aluminum  
75 or the aluminum alloy into the melting  
chamber, then melting the aluminum or the  
aluminum alloy in this atmosphere which is  
substantially chemically inert toward the  
aluminum or the aluminum alloy, and then  
80 creating a partial vacuum within the said  
melting chamber while the aluminum or the  
aluminum alloy is yet molten.

4. The process of melting aluminum or an  
aluminum alloy which consists in creating a  
partial vacuum within the melting chamber,  
then admitting into the melting chamber a  
reagent which has the property of combin-  
ing with the oxygen present within the melt-  
ing chamber thereby producing an atmos-  
phere within the melting chamber which is  
85 substantially chemically inert toward the  
aluminum or the aluminum alloy and then  
melting the aluminum or the aluminum  
alloy in this atmosphere which is substan-  
tially chemically inert toward the aluminum  
or the aluminum alloy.

Signed at New York city in the county of  
New York and State of New York this 9th  
day of February A. D. 1911.

GRENVILLE MELLEN.

Witnesses:

FRED. F. KUHLMANN,  
S. R. MILLER.

Copies of this patent may be obtained for five cents each, by addressing the "Commissioner of Patents,  
Washington, D. C."